# EUROPEAN PATENT SPECIFICATION

(11) **EP 2 041 738 B1**
(45) Date of publication and mention of the grant of the patent: **12.03.2014**
(21) Application number: 07798725.3
(22) Date of filing: 19.06.2007
(51) Int. Cl.: G09F 3/02, B44C 3/02

(54) **DISPLAYING PRINTED IMAGES ON IRREGULAR SUBSTRATES**
ANZEIGE VON DRUCKBILDERN AUF UNREGELMÄSSIGEN SUBSTRATEN
AFFICHAGE D'IMAGES IMPRIMÉES SUR DES SUBSTRATS IRRÉGULIERS

(30) Priority: 29.06.2006 US 427398
(43) Date of publication of application: 01.04.2009
(73) Proprietor: 3M Innovative Properties Company, St. Paul, MN 55133-3427 (US)
(72) Inventor: STEELMAN, Ronald, S., Saint Paul, MN 55133-3427 (US)
(74) Representative: Vossius & Partner
(86) International application number: PCT/US2007/071508
(87) International publication number: WO 2008/002794

(56) References cited:
- WO-A1-00/43220
- WO-A1-97/33947
- KR-A- 20030 036 639
- US-A- 5 034 077
- US-A- 5 284 689
- US-A1- 2004 191 664
- US-A1- 2006 063 673
- US-B1- 6 270 871
- US-B1- 6 709 726
- US-B2- 6 663 947

## Description

### Background

The present disclosure relates generally to displaying graphics on irregular substrates.

Adhesive-coated plastic films, especially vinyl films with pressure sensitive adhesives or pressure-activated adhesives, are applied to a variety of surfaces for a variety of reasons such as advertisement, decoration, protection, and the like. Most of these surfaces tend to be fairly smooth. However, there are many surfaces that are non-planar or irregular and may include imperfections, seams, rivets, and other protrusions or indentations.

When a film is applied over and adhered to these irregular surfaces, the film may be strained to bring the adhesive into contact with the irregular surface. Residual stress in the film at such irregular surface locations may exceed the holding power of the adhesive resulting in the film lifting off the surface to which it was adhered. This may result in an imperfect appearance.

WO 00/43220 describes a method of applying adhesive coated film, wherein adhesive coated film is applied to a surface, especially an irregular surface by use of heat and a heat-neutral pressure source.

WO 97/33947 describes heat activated, translucent marking films having a transferable, translucent, plastic film and field of a heat activated, translucent adhesive adhered to the plastic film.

### Summary

In an illustrative but non-limiting example of the disclosure, method of displaying a printed image on an irregular substrate as defined in independent claim 1 is disclosed. A polymer film having a glass transition temperature of at least 40°C is provided. The polymer film has an adhesive layer disposed on a second side of the film. An image may be printed on a first side of the film with a solvent-based ink. The adhesive layer may be positioned against the irregular substrate such that the polymer film at least partially bridges irregularities in the irregular substrate and the polymer film may be heated. The heated polymer film is pressed against the irregular substrate such that much of the adhesive layer comes into contact with the irregular substrate.

In another illustrative but non-limiting example of the disclosure, a method of adhering a printed image onto an irregular substrate as defined in independent claim 5 is disclosed. An image may be printed onto a polymer film having a glass transition temperature of at least about 40°C using a solvent-based ink. An adhesive layer may be disposed on the polymer film. The polymer film may be positioned such that the adhesive layer at least partially contacts the irregular substrate. The polymer film may be heated to form a softened film, which may then be pressed into the irregular substrate so that most of the film comes into contact with the irregular substrate.

In another illustrative but non-limiting example of the disclosure, an assembly as defined in independent claim 12 is disclosed. The assembly includes an irregular substrate and an adhesive layer that is substantially in intimate contact with the irregular substrate. A polymer film having a glass transition temperature of at least about 40°C may be in intimate contact with the adhesive layer. A piezo inkjet ink image may be printed onto the polymer film.

The above summary of the disclosure is not intended to be all-encompassing. Other details of the disclosure will be evident to those of ordinary skill in the art from the following detailed description together with the drawings.

### Brief Description of the Drawings

The disclosure may be more completely understood in consideration of the following detailed description of the accompanying drawings, in which:
Figure 1 is a schematic view of an illustrative but non-limiting irregular substrate as described herein;
Figure 2 is a schematic view of an illustrative but non-limiting laminate applied in partial contact with the irregular substrate of Figure 1;
Figure 3 is a schematic view of an illustrative but non-limiting laminate in intimate contact with the irregular substrate of Figure 1;
Figure 4 is a schematic view of an illustrative but non-limiting laminate as described herein;
Figure 5 is a schematic view of an illustrative but non-limiting laminate as described herein; and
Figure 6 is a schematic view of an illustrative but non-limiting laminate as described herein.

### Detailed Description

Unless otherwise indicated, all numbers expressing feature sizes, amounts, and physical properties used in the specification and claims are to be understood as being modified in all instances by the term "about." Accordingly, unless indicated to the contrary, the numerical parameters set forth in the foregoing specification and attached claims are approximations that can vary depending upon the desired properties sought to be obtained by those skilled in the art utilizing the teachings disclosed herein.

The recitation of numerical ranges by endpoints includes all numbers subsumed within that range (e.g. 1 to 5 includes 1, 1.5, 2, 2.75, 3, 3.80, 4, and 5) and any range within that range.

As used in this specification and the appended claims, the singular forms "a", "an", and "the" encompass embodiments having plural referents, unless the content clearly dictates otherwise. For example, reference to "a layer" encompasses embodiments having one, two or more layers. As used in this specification and the appended claims, the term "or" is generally employed in its sense including "and/or" unless the content clearly dictates otherwise.

The term "polymer" will be understood to include polymers, copolymers (e.g., polymers formed using two or more different monomers), oligomers and combinations thereof, as well as polymers, oligomers, or copolymers that can be formed in a miscible blend.

The disclosure pertains to displaying images such as printed images on an irregular substrate. An irregular substrate may include a non-planar surface. In some instances, an irregular substrate may include a planar or substantially planar surface and one or more non-planar elements that are disposed on or in the planar surface. Some or all of the non-planar elements may extend into, or below, the planar surface. Some or all of the non-planar elements may extend above the planar surface.

In some instances, the irregular substrate may be a building or construction substrate, such as a wall. Examples of irregular substrates include masonry such as concrete and brick and stone. The irregular substrate may be a metallic substrate, such as a side of a truck or trailer. In some instances, the side of a truck or trailer may be curved. In some cases, the side of a truck or trailer may be substantially planar, with non-planar elements such as seams, rivets, screw heads and the like.

The disclosure pertains to printing an image on a polymer film that may subsequently be secured to the irregular substrate. Any suitable polymer film may be used. In some instances, the polymer film may be made from a material having a glass transition temperature of at least about 40°C. In some cases, the polymer film may be made from a material having a glass transition temperature of at least about 60°C or even at least about 80°C. It should be recognized that some polymeric materials may have more than one glass transition temperature, or temperature at which portions of the polymer may soften. For the purposes of referring to glass transition temperature herein, it is intended that the temperature in question for a particular material is the temperature at which the entire material has softened. i.e. the last or final glass transition temperature.

The polymer film may have a thickness of about 25 micrometers to about 100 micrometers. In some instances, the polymer film may be at least substantially transparent to visible light.

Examples of suitable polymers include polyvinyl chloride, poly(meth)acrylate films such as poly(methyl methacrylate), polyester films, polycarbonate sheets, styrene sheets and the like.

An adhesive layer such as a pressure sensitive adhesive may be applied to the polymer film to adhere the polymer film to the irregular substrate. Any suitable pressure sensitive adhesive may be used, providing the particular pressure sensitive adhesive used has adequate adherence to both the polymer film and the irregular substrate to which the adhesive layer will be secured. In some instances, the pressure sensitive adhesive may be at least substantially transparent to visible light. A transparent adhesive may be used, for example, if the polymer film is also transparent, and it is desired that the irregular substrate be visible through the adhesive and the polymer film.

In some cases, the pressure sensitive adhesive may be pigmented to appear a particular color. For example, the pressure sensitive adhesive may include titanium dioxide, and thus will appear white. A white-tinted adhesive may be applied to a substantially clear polymer film, for example, to provide a largely white backdrop for a printed image. In some instances, the pigmented adhesive may be laminated to the imaged side of the polymer film such that the polymer film serves as a protective layer for the image after the adhesive is attached to a irregular substrate. Suitable pigments for achieving other colors, such as yellow, orange, green, blue, red and the like are known.

A variety of pressure sensitive adhesives (PSAs) are useful. Pressure sensitive adhesives may be defined as material with the following properties: (1) aggressive and permanent tack, (2) adherence with no more than finger pressure, (3) sufficient ability to hold onto an adherand, (4) sufficient cohesive strength, and (5) require no activation by an energy source. Useful PSAs may exhibit pressure sensitive adhesive characteristics at either room temperature or at elevated temperatures.

PSAs are normally tacky at assembly temperatures, which is typically room temperature or greater (i.e., about 20°C to about 90°C or greater). Materials that have been found to function well as PSAs are polymers designed and formulated to exhibit the requisite viscoelastic properties resulting in a desired balance of tack, peel adhesion, and shear holding power at the assembly temperature and also retain properties such as peel adhesion and shear holding power at ambient temperatures.

Examples of polymers useful in preparing pressure sensitive adhesives include natural rubber-, synthetic rubber- (e.g., styrene/butadiene copolymers (SBR) and styrene/isoprene/styrene (SIS) block copolymers), silicone elastomer-, poly alpha-olefin-, and various (meth) acrylate- (e.g., acrylate and methacrylate) based polymers. Of these, (meth)acrylate-based polymer pressure sensitive adhesives are useful as a result of their optical clarity, permanence of properties over time (aging stability), and versatility of adhesion levels, to name just a few of their benefits.

In some instances, a release liner may be provided on the adhesive layer. The release liner can be formed of any useful material such as, for example, polymers or paper and may include a release coat. Suitable materials for use in release coats are well known and include, but are not limited to, fluoropolymers, acrylics and silicones designed to facilitate the release of the release liner from the pressure sensitive adhesive. The release coat may be designed to remain substantially adhered to the release liner after the transfer of the film to the surface to be finished.

The disclosure pertains to displaying an image that has been printed onto a polymer film. In some instances, an image may be printed onto the polymer film using organic solvent-based printing, which may also be referred to as piezo printing. Solvent-based printing may be accomplished using a variety of commercially available piezo inkjet printers. Examples of suitable printers include those available from Idanit Technologies, Ltd. of Rishon Le Zion Israel, Raster Graphics of San Jose, Calif., Vutek Inc. of Meredith, N.H., Olympus Optical Co. Ltd. of Tokyo, Japan, and others.

Piezo inkjet printing principally relies on the use of four colors: cyan, magenta, yellow, and black (CMYK). However, to improve the resolution of images, some printers identified above also add two additional colors that are less concentrated relatives of the cyan and magenta inks, called "light cyan" and "light magenta." Additionally, printers and software can be configured to use "special" or "spot" colors that are specific hues based on large usage or commercial branding requirements.

A useful solvent-based piezo ink may include a pigment, a binder, an optional plasticizer, an organic solvent, a surfactant, and an antifoaming agent. Each of these components is described in greater detail hereinafter, and also in U.S. Patent No. 6,379,444.

Organic solvents suitable for use in the inks described herein include ketones, aromatic hydrocarbons, ethers and esters (e.g., lactates, acetates, etc.). Examples of such solvents include cyclohexanone, propylene glycol monomethyl ether acetate (PM acetate), diethylene glycol ethyl ether acetate (DE acetate), isophorone, ethylene glycol butyl ether acetate (EB acetate), dipropylene glycol monomethyl acetate (DPM acetate), butyrol lactone, n-methyl pyrrolidone, alkyl acetate esters (such as those available under the trade designations EXXATE 600, EXXATE 700, and EXXATE 800 fluids from ExxonMobil Corp., Irving, Tex.), and combinations thereof.

Fluorochemical surfactants may act as a flow agent to lower the surface tension of solvents. The lower surface tension allows the inks to flow out better on the receiving substrate. Such fluorochemical surfactants are solutes in solvents used in the present invention. Non-limiting examples of fluorochemical surfactants include the family of FC branded chemicals from 3M Company and preferably includes FLUORAD FC430 and FC431. Such chemicals are fluorinated alkyl esters. Silicone and other organic surfactants may also be used.

The antifoaming agent includes an antifoaming oil and preferably a particulate material. The antifoaming agent may be dispersed in solvents to aid in minimizing foaming that might otherwise be caused by the fluorochemical surfactants. Antifoaming oils may be viscous, substantially water-insoluble liquids that can alter the surface tension of a fluid at room temperature. Silicone and other organic anti-foaming materials may also be used.

Piezo inks include one or more colorants, such as a pigment. A pigment can be an inorganic or organic, colored, white or black material that is practically insoluble in the medium (e.g., organic solvent) in which it is incorporated. Examples of suitable pigments include those useful in screen printing. An ink may include only one color pigment, or may include several different pigments to achieve a desired color. A variety of pigments are available. In some instances, an ink may also include one or more dyes.

Non-limiting examples of cyan pigments include IRGALITE GLG (Ciba Specialty Chemicals of Greensboro, N.C.) and SUNFAST 249-1284 (Sun Chemical Corporation of Fort Lee, N.J.). Non-limiting examples of magenta pigments include QUINDO magenta RV-6828 (Bayer of Pittsburgh, Pa.) and Magenta B RT-343-D (Ciba Specialty Chemicals). Non-limiting examples of yellow pigments include Fanchon Fast yellow Y5686 (Bayer) Fanchon yellow Y5688 (Bayer), and Sandorin 6GL (Clariant of Charlotte, N.C.). Non-limiting examples of black pigments include Pfizer lampblack LB-1011 (Pfizer of Easton, Pa.) and Raven 1200 (Columbian Chemicals of Atlanta, Ga.).

Piezo inks may include binders. A binder can be a resin that is compatible with pigment particles such that upon evaporation of volatile components of the ink, the binders form films of the deposited pigments on the receiving substrate. Advantageously, the binders described herein are outdoor durable. Non-limiting examples of suitable binders are polymeric resins such as vinyl-containing polymers (e.g, VYHH, VYNS, VYHD, and VAGH brand vinyl-containing resins from Union Carbide) and acrylic-containing polymers (e.g., polymethylmethacrylate, polymethylbutylacrylate, polyethylmethacrylate and copolymers thereof).

For some applications, it may be desirable that the inks are radiation curable. For example, radiation curable inks may be prepared by incorporating radiation curable materials including, but not limited to, monomers, oligomers, stabilizers, and optionally initiators and pigments into the ink. After the resulting inks have been applied to a receptor, they may be cured by exposure to radiation such as electron beam (e-beam) radiation. If photoinitiators or photocatalysts are also incorporated into the radiation curable inks, the resulting inks may be cured after they have been applied to a receptor by exposure to actinic radiation such as ultraviolet (UV) or visible-light.

The optional plasticizers may be polyesters that are compatible with the vinyl and acrylic resins and any other binder used along with the stabilizers and flow agents such that upon evaporation of volatile components of the ink, the plasticizers enhance the flexibility of the film formed from the deposited binder with pigments on the receiving substrate. The plasticizer also becomes part of the final ink film. Non-limiting examples of suitable plasticizers include UNIFLEX 312 brand plasticizer (Union Camp of Wayne, N.J.), PARAPLEX G-31 brand plasticizer (C. P. Hall of Chicago, Ill.) and PARAPLEX G-51 brand plasticizer (C. P. Hall).

To enhance durability of a printed image graphic, especially in outdoor environments exposed to sunlight or moisture, a variety of commercially available stabilizing chemicals can be added optionally to inks of the present invention. These stabilizers may include heat stabilizers, UV light stabilizers and biocides.

Heat stabilizers are commonly used to protect the resulting image graphic against the effects of heat and are commercially available as Mark V1923 brand stabilizer (Witco of Houston, Tex.), Synpron 1163 brand stabilizer (Ferro of Cleveland, Ohio), Ferro 1237 brand stabilizer (Ferro), and Ferro 1720 brand stabilizer (Ferro). UV light stabilizers are commercially available as UVINOL 400 brand benzophenone uv-absorber (BASF of Parsippany, N.J.) and TINUVIN 900 brand uv-absorber (Ciba Specialty Chemicals). An example of a commercially available biocide is VINYZENE SB-1 EAA Antimicrobial Additive for Plastics, available from Morton Thiokol, Inc.

The following description should be read with reference to the drawings, in which like elements in different drawings are numbered in like fashion. The drawings, which are not necessarily to scale, depict selected illustrative embodiments and are not intended to limit the scope of the disclosure. Although examples of construction, dimensions, and materials are illustrated for the various elements, those skilled in the art will recognize that many of the examples provided have suitable alternatives that may be utilized.

Figure 1 provides a schematic illustration of an irregular substrate 10 that may, as noted above, represent a building material, a vehicle or some other irregular surface upon which it may be desired to apply a printed image. The irregular substrate 10 may be seen as including a planar surface 12 and non-planar elements including protrusions 14 and indentations 16. The protrusions 14 may be considered as extending out of the plane of the planar surface 12 while the indentations 16 may be considered as extending into the plane of the planar surface 12.

It will be recognized, of course, that in some instances the irregular substrate 10 may include the protrusions 14 but not include any of the indentations 16. In other cases, the irregular substrate 10 may include indentations 16 but not include any protrusions 14. It will also be recognized that protrusions 14 and indentations 16, as illustrated, are highly stylized. In some cases, the protrusions 14 may represent rivets, screw heads, bolt heads, welding materials, seams, and the like. In some cases, the indentations 16 may represent dents, screw or bolt holes lacking a screw or bolt, and the like. If the irregular substrate 10 is masonry or stone, the protrusions 14 and/or the indentations 16 may represent grout lines, imperfections, voids, protruding particles and the like in the material.

In Figure 2, a laminate 18 has been positioned proximate the irregular substrate 10. The laminate 18 includes a polymer film 20 having, as illustrated, a printed image 22 formed on a first side 24 of the polymer film 20 and an adhesive layer 26 disposed on an opposing second side 28 of the polymer film 20. The printed image 22 may be formed using organic solvent-based printing, as described above. The adhesive layer 26 may include any suitable pressure sensitive adhesive, as described above. As illustrated, it is considered that the adhesive layer 26 makes sufficient contact with at least a portion of the irregular substrate 10 to hold the laminate 18 in position. The adhesive layer 26 may be considered as being in partial contact with the irregular substrate 10.

To fully apply the laminate 18 to the irregular substrate 10, as shown in Figure 3, it may be useful to heat the laminate 18, at least to soften the polymer film 20. Any suitable heat source may be used, provided the heat source can provide sufficient thermal energy to soften the polymer film 20 without causing the polymer film 20 to reach or exceed its melting point. In some instances, a heat source such as a heat gun that is capable of providing 1000°F (about 540°C) may be used. A heat source generating infrared energy may be used. A combination of hot air and infrared heat, such as generated by a catalytic heater may be used. It is considered that in some instances, all or substantially all of the polymer film 20 may be heated at once. In some cases, particularly if the laminate 18 is quite large, it may be useful to only heat a portion of the polymer film 20 at a time.

Once the polymer film 20, or a portion thereof, has been heated sufficiently to soften the polymer film 20, the softened film 20 may be pressed against or into the irregular substrate 10 such that the adhesive layer 26 makes intimate contact with the irregular substrate 10. Pressure may be applied to the laminate 18 using any appropriate technique or device. In some cases, it may be useful to use a roller, block or brush to push and/or rub the laminate 18 onto the irregular substrate 10. A roller, block or brush may be formed from a material such as natural or synthetic rubber, urethane polymers, silicone polymers, fluoroelastomers, foamed or sponge versions of those rubbers, and the like. An open cell foamed silicone material having cells that are no larger than about 0.5 millimeters is particularly useful

It may be useful to use a roller or such that is formed from a material having a relatively low thermal conductivity such that the roller, block or brush does not, itself, remove too much thermal energy from the heated, softened laminate 18. Instead, it is desired that the polymer film 20 remain softened until the adhesive layer 26 makes intimate contact with the irregular substrate 10. Once the adhesive layer 26 makes intimate contact with the irregular substrate 10, it is considered that the irregular substrate 10, being at or close to ambient temperature, will draw sufficient thermal energy out of the laminate 18 to permit the polymer film 20 to harden and thus permanently assume the profile of the irregular substrate 10.

Figures 2 and 3 provide an example of displaying a printed image on an irregular substrate 10 using a laminate 18. It will be recognized that the laminate 18 may be formed in several different ways, and may take several different forms. The subsequent Figures represent laminates that may be used in displaying a printed image on the irregular substrate 10.

Figure 4 shows a laminate 30 that includes a polymer film 32 having a first side 34 and a second side 36. An adhesive layer 38 is disposed on the second side 36. While not required, a release liner 40, as discussed above, may be disposed on the adhesive layer 38 to protect the adhesive layer 38 and also to prevent undesired adhesion during printing. An image 42 may be printed on the first side 34 using a solvent-based ink after the adhesive layer 38 is applied or otherwise disposed on the second side 36. In some cases, the solvent-based ink may penetrate a short distance into the first side 34 of the polymer film 32. In some instances, the solvent-based ink does not penetrate into the polymer film 32. The laminate 30 may then be applied to an irregular substrate 10 (Figure 1) as described above.

In some instances, an adhesive layer may be applied after the polymer film has been printed, as shown for example in Figures 5 and 6. In particular, Figure 5 shows a laminate 44 that includes a polymer film 46 having a first side 48 and a second side 50. A printed image 52 may be printed onto the first side 48 of the polymer film 46. An adhesive layer 54 may subsequently be disposed on the second side 50 of the polymer film 46. If desired, a release liner (not shown) may be applied over the adhesive layer 54. The laminate 44 may then be applied to an irregular substrate 10 (Figure 1) as described above.

Figure 6 illustrates a laminate 56 in which an adhesive layer and a printed image are formed on a single side of a polymer film. Such a laminate 56 may, for example, provide additional protection for the printed image. The laminate 56 includes a polymer film 58 having a first side 60 and a second side 62. The polymer film 58 may be at least substantially transparent to visible light. The second side 62 may, once the laminate 56 is applied, be the exterior or exposed side of the polymer film 58.

A printed image 64 may be formed on the first side 60 of the polymer film 58. It will be recognized that the printed image 64 may, if desired, be printed in a mirror-image fashion so that the image appears correctly oriented when viewed through the polymer film 58 from the second side 62 thereof. The printed image 64 may be formed using solvent-based printing, as discussed above.

Once the printed image 64 has been formed, an adhesive layer 66 may be formed or otherwise disposed over the printed image 64. The adhesive layer 66 may include any suitable adhesive such as a pressure sensitive adhesive. The adhesive layer 66 may, as discussed above, include pigments to provide a desired background color for the printed image 64. As a result, the printed image 64 does not have to cover an entire surface of the polymer film 58 as the background color provided by the adhesive layer 66 may contribute to the aesthetics of the laminate 56. The laminate 56 may then be applied to the irregular substrate 10 (Figure 1) as discussed above.

The present invention should not be considered limited to the particular examples described herein, but rather should be understood to cover all aspects of the invention as fairly set out in the attached claims. Various modifications, equivalent processes, as well as numerous structures to which the present invention can be applicable will be readily apparent to those of skill in the art to which the present invention is directed upon review of the instant specification.

### EXAMPLES

Example 1 was prepared using a polyvinyl chloride (PVC) film about 25 cm x 10 cm and 0.004 inches (0.1 mm) thick; available from Klöckner Pentaplast of America, Inc., Gordonsville, VA. The film had a glass transition midpoint temperature when tested by Differential Scanning Calorimeter (DSC) of 79°C.

glass transition temperature of film specimens was measured by weighing and loading the specimens into TA Instruments aluminum standard DSC sample pans. The specimens were analyzed using the TA Instruments Q1000 (#131, Cell RC-858) Modulated^{®} Differential Scanning Calorimeter (MDSC). The modulated method used to analyze the samples included a linear heating rate of 5°C/min. plus an applied perturbation amplitude of ±0.796°C every 60 seconds. The specimens were subjected to a heat-cool-heat profile over a temperature range of -100 to about 175°C. The glass transition temperatures reported were evaluated using the step change in the reversing (R) heat flow (heat capacity related) curve. The onset, midpoint (half height), and end temperatures of the transition are noted, and the midpoint is the stated value.

The PVC film was coated on one side with an acrylic pressure sensitive adhesive having a dried thickness of 0.0015 inches (0.04 mm). The adhesive composition was 96 wt-% 2-methylbutyl acrylate and 4 wt-% acrylamide that was crosslinked using UV light and a benzophenone photoinitiator in a manner similar to that described in US Patent 4,181,752. The adhesive was coated on a silicone release liner and then transferred to the PVC film described above.

A controlled textured surface panel was prepared by laminating Regal Resin Bond Cloth Open Coat 960G, 36 grit YN sandpaper obtained from 3M Company, St. Paul, MN to a plywood panel using a standard contact cement. This surface has low affinity for pressure sensitive adhesives, is very consistent compared to typical textures surfaces for which this product is most suited, and it has a similar profile to a typical sand stucco surface. Lower adhesion to the surface is desired because the pressure sensitive adhesive composition influences the apparent conformability of the film. A very good pressure sensitive adhesive and/or a surface that bonds readily to the pressure sensitive adhesive can delay the onset of lifting when used with films that have a glass transition below 40°C and use the method described herein.

The release liner was removed from the film. The adhesive coated side of the film was loosely placed using hand pressure against the textured surface panel such that the adhesive was contacting the panel and there was sufficient adhesion for the film to temporarily remain attached to the panel, but in most areas, the film was bridging indentations in the panel.

A Steinel heat gun (Model HG3002LCD; available from McMaster Carr, (600 County Line Rd., Elmhurst, IL 60126-2081) was set at 1000°F (538°C). The heat gun was held about 2 inches (5 cm) from the film surface with heating of the film in one area until the film visibly softened. Heating of the film was immediately followed by use of a 3M TSA-1 Textured Surface Applicator available from Commercial Graphics Division, 3M Company to firmly roll the film with hand pressure at about 4 inches (10 cm) per second onto the textured surface of the panel. The heat gun was moved across the film sample followed immediately by roll down of the film with the applicator.

After rolling the film against the textured surface of the panel, the film immediately cooled to the panel temperature. The film was intimately bonded to the panel and looked similar to a painted surface. The gloss of the film bonded to the panel was measured using a BYK Gardner 60° micro gloss meter (Model No 4501.; available from BYK Gardner USA, 2435 Linden Lane, Silver Spring, MD) and recorded. The panel was then placed in a 150°F (65°C) oven for 24 hours, removed from the oven and allowed to cool to ambient temperature and the gloss of the film measured and recorded.

Example 2 was prepared as described for Example 1, except using a clear acrylic KORAD™ film available from Spartech PEP. The film was about 25 cm x 10 cm and was 0.003 inches (0.8 mm) thick. The film had a glass transition midpoint temperature when tested as described above by Differential Scanning Calorimeter (DSC) of 79°C.

The release liner was removed from the KORAD film, the film was applied to the textured surface panel, and the gloss of the film was measured as described for Example 1.

Comparative Example 1 was 3M™ Controltac™ Plus Graphic film Series 180-10 (50 micrometer thick white vinyl film with about 30 micrometers of adhesive; "180 Vinyl Film"; 3M Company). The sample size was 25 cm x 10 cm and the glass transition temperature measured as described for Example 1 was 19°C. Gloss measurements were taken and recorded as described for Example 1.

Provided in Table 1 are the gloss measurements of the film samples of Examples 1 and 2 prior to application of the adhesive and the sample of 180 Vinyl Film (Initial), immediately after application of the samples to the textured surface panel and after heating in a 65°C (150°F) oven for 24 hours. The data in Table 1 are the mean of 18 readings at different locations on the film for each sample initially, immediately after application and after 24 hour heat aging. The standard deviations are proved in parentheses after the readings.

The actual gloss values are the mean +/- 3 standard deviation units. Since individual films vary slightly in gloss, the value for comparison is a percentage of original gloss and the standard deviation for comparison is 100/initial film gloss multiplied by the measured standard deviation. The adjusted gloss values provided in Table 1 are based on 100/original gloss multiplied by the measured value.

| Time of Measurement | Example1 | Example 2 | Comparative Example 1 |
|---|---|---|---|
| | Actual Gloss Values | | |
| Initial | 82.6 | 144 | 80.7 |
| Immediately After Application | 5.2 (1.0) | 5.1 (0.8) | 4.0 (0.8) |
| After 24 Hour Heat Aging | 5.3 (1.2) | 8.8 (4.0) | 9.4 (5.0) |
| | | | |

| | Adjusted Gloss Values | | |
|---|---|---|---|
| Immediately After Application | 6.3 (1.2) | 3.6 (.6) | 5.0 (1.0) |
| After 24 Hour Heat Aging | 6.4 (1.5) | 6.1 (2.8) | 11.6 (6.2) |

The data in Table 1 show that the film of Example 1 maintained substantially the same gloss value after heat aging, whereas the film of Comparative Example 1 showed a marked increase in gloss value. While the film of Example 2 showed a greater increase in adjusted gloss value than that of Example 1, the change in adjusted gloss value was still much less than the film of Comparative Example 1. Upon visual inspection, it was observed that areas of the film of Comparative Example 1 had lifted off the textured surface panel and had become planar. In general, lower gloss indicates better compliance to the textured surface panel, provided the surface finish of the film has not been damaged by the application process.

Illustrative embodiments of this disclosure are discussed and reference has been made to possible variations within the scope of this disclosure. These and other variations and modifications in the disclosure will be apparent to those skilled in the art without departing from the scope of the disclosure, and it should be understood that this disclosure is not limited to the illustrative embodiments set forth herein. Accordingly, the disclosure is to be limited only by the claims provided below, and as they may be amended during prosecution.

## Claims

1. A method of displaying a printed image on an irregular substrate (10) having a non-planar surface, the method comprising steps of:
providing a polymer film (20) having a glass transition temperature of at least 40°C, the polymer (20) film having a first side (24) and a second side (28), an adhesive layer (26) disposed on the second side (28), wherein the adhesive is a pressure sensitive adhesive that is tacky at assembly temperatures;
printing an image (22) with a solvent-based ink on the first side (24);
positioning the adhesive layer (26) against the irregular substrate (10);
heating the polymer film (20); and
pressing the heated polymer film (20) against the irregular substrate (10).

2. The method of claim 1, wherein the polymer film (20) has a glass transition temperature of at least 60°C.

3. The method of claim 1, wherein the polymer film (20) comprises a polyvinyl chloride film or a polymethyl methacrylate film.

4. The method of claim 1, wherein the irregular substrate comprises a planar surface and non-planar surface elements.

5. A method of adhering a printed image onto an irregular substrate (10) having a non-planar surface, the method comprising steps of:
printing an image (22) with a solvent-based ink onto a polymer film (20) having a glass transition temperature of at least 40°C;
disposing an adhesive layer (26) on the polymer film (20);
positioning the polymer film (20) on an irregular substrate (10) such that the adhesive contacts the irregular substrate (10);
heating the polymer film (20) to form a softened film; and
pressing the softened film into the irregular substrate (10),
wherein the adhesive is a pressure sensitive adhesive that is tacky at assembly temperatures.

6. The method of claim 5, wherein the adhesive layer (26) is pigmented.

7. The method of claim 5, wherein the adhesive layer (26) is optically transparent.

8. The method of claim 5, wherein the film (20) is optically transparent.

9. The method of claim 5, wherein attaching the polymer film (20) onto the irregular substrate (10) comprises making only partial contact between the adhesive layer (26) and the irregular substrate (10).

10. The method of claim 5, wherein printing an image (22) with a solvent-based ink comprises inkjet printing with a solvent-based ink.

11. The method of claim 65 wherein the irregular substrate comprises a planar surface (12) and non-planar surface elements (14, 16).

12. An assembly, comprising:
an irregular substrate (10) having a non-planar surface;
an adhesive layer (26) in contact with the irregular substrate (10);
a polymer film (20) in contact with the adhesive layer (26), the polymer film (20) having a glass transition temperature of at least 40°C; and
a piezo inkjet ink image (22) printed onto the polymer film (20),
wherein the adhesive is a pressure sensitive adhesive that is tacky at assembly temperatures.

13. The assembly of claim 12, wherein the polymer film (20) has a glass transition temperature of at least 80°C.

## Patentansprüche

1. Verfahren zum Anzeigen eines Druckbilds auf einem unregelmäßigen Substrat (10), das eine nichtplanare Oberfläche aufweist, wobei das Verfahren die Schritte umfasst des:
Bereitstellens einer Polymerfolie (20), die eine Glasübergangstemperatur von mindestens 40 °C aufweist, wobei die Polymerfolie (20) eine erste Seite (24) und eine zweite Seite (28), eine Klebstoffschicht (26), die sich auf der zweiten Seite (28) befindet, aufweist, wobei der Klebstoff ein Haftklebstoff ist, der bei Zusammenbautemperaturen klebrig ist,
Druckens eines Bilds (22) mit einer Tinte auf Lösungsmittelbasis auf die erste Seite (24);
Positionierens der Klebstoffschicht (26) gegen das unregelmäßige Substrat (10);
Erhitzens der Polymerfolie (20); und
Drückens der erhitzten Polymerfolie (20) gegen das unregelmäßige Substrat (10).

2. Verfahren nach Anspruch 1, wobei die Polymerfolie (20) eine Glasübergangstemperatur von mindestens 60 °C aufweist.

3. Verfahren nach Anspruch 1, wobei die Polymerfolie (20) eine Polyvinylchloridfolie oder eine Polymethylmethacrylatfolie umfasst.

4. Verfahren nach Anspruch 1, wobei das unregelmäßige Substrat eine planare Oberfläche und nichtplanare Oberflächenelemente aufweist.

5. Verfahren zum Befestigen eines Druckbilds auf einem unregelmäßigen Substrat (10), das eine nichtplanare Oberfläche aufweist, wobei das Verfahren die Schritte umfasst des:
Druckens eines Bilds (22) mit einer Tinte auf Lösungsmittelbasis auf eine Polymerfolie (20), die eine Glasübergangstemperatur von mindestens 40 °C aufweist;
Aufbringens einer Klebstoffschicht (26) auf die Polymerfolie (20);
Positionierens der Polymerfolie (20) auf ein unregelmäßiges Substrat (10), derart, dass der Klebstoff das unregelmäßige Substrat (10) kontaktiert;
Erhitzens der Polymerfolie (20), um eine erweichte Folie zu bilden; und
Drückens der erweichten Folie in das unregelmäßige Substrat (10),
wobei der Klebstoff ein Haftklebstoff ist, der bei Zusammenbautemperaturen klebrig ist.

6. Verfahren nach Anspruch 5, wobei die Klebstoffschicht (26) pigmentiert ist.

7. Verfahren nach Anspruch 5, wobei die Klebstoffschicht (26) optisch transparent ist.

8. Verfahren nach Anspruch 5, wobei die Folie (20) optisch transparent ist.

9. Verfahren nach Anspruch 5, wobei das Anbringen der Polymerfolie (20) an das unregelmäßige Substrat (10) das Herstellen von nur teilweisem Kontakt zwischen der Klebstoffschicht (26) und dem unregelmäßigen Substrat (10) umfasst.

10. Verfahren nach Anspruch 5, wobei das Drucken eines Bilds (22) mit einer Tinte auf Lösungsmittelbasis das Tintenstrahldrucken mit einer Tinte auf Lösungsmittelbasis umfasst.

11. Verfahren nach Anspruch 5, wobei das unregelmäßige Substrat eine planare Oberfläche (12) und nichtplanare Oberflächenelemente (14, 16) umfasst.

12. Zusammenbau, umfassend:
ein unregelmäßiges Substrat (10), das eine nichtplanare Oberfläche aufweist;
eine Klebstoffschicht (26) in Kontakt mit dem unregelmäßigen Substrat (10);
eine Polymerfolie (20) in Kontakt mit der Klebstoffschicht (26), wobei die Polymerfolie (20) eine Glasübergangstemperatur von mindestens 40 °C aufweist; und
ein Piezo-Tintenstrahltintenbild (22), das auf die Polymerfolie (20) aufgedruckt ist,
wobei der Klebstoff ein Haftklebstoff ist, der bei Zusammenbautemperaturen klebrig ist.

13. Zusammenbau nach Anspruch 12, wobei die Polymerfolie (20) eine Glasübergangstemperatur von mindestens 80 °C aufweist.

## Revendications

1. Procédé d'affichage d'une image imprimée sur un substrat irrégulier (10) comportant une surface non plane, le procédé consistant à :
fournir un film de polymère (20) ayant une température de transition vitreuse d'au moins 40 °C, le film de polymère (20) comportant un premier côté (24) et un deuxième côté (28), une couche d'adhésif (26) étant disposée sur le deuxième côté (28), et l'adhésif étant un adhésif sensible à la pression qui est collant aux températures d'assemblage ;
imprimer une image (22) avec une encre à base de solvant sur le premier côté (24) ;
positionner la couche d'adhésif (26) contre le substrat irrégulier (10) ;
chauffer le film de polymère (20) ; et
presser le film de polymère (20) chauffé contre le substrat irrégulier (10).

2. Procédé selon la revendication 1, dans lequel le film de polymère (20) a une température de transition vitreuse d'au moins 60 °C.

3. Procédé selon la revendication 1, dans lequel le film de polymère (20) comprend un film de polychlorure de vinyle ou un film de polyméthacrylate de méthyle.

4. Procédé selon la revendication 1, dans lequel le substrat irrégulier comprend une surface plane et des éléments de surface non plans.

5. Procédé pour faire adhérer une image imprimée sur un substrat irrégulier (10) comportant une surface non plane, le procédé consistant à :
imprimer une image (22) avec une encre à base de solvant sur un film de polymère (20) ayant une température de transition vitreuse d'au moins 40 °C;
disposer une couche d'adhésif (26) sur le film de polymère (20) ;
positionner le film de polymère (20) sur un substrat irrégulier (10) de telle sorte que l'adhésif entre en contact avec le substrat irrégulier (10) ;
chauffer le film de polymère (20) pour former un film ramolli ; et
presser le film ramolli contre le substrat irrégulier (10).
l'adhésif étant un adhésif sensible à la pression qui est collant aux températures d'assemblage.

6. Procédé selon la revendication 5, dans lequel la couche d'adhésif (26) est pigmentée.

7. Procédé selon la revendication 5, dans lequel la couche d'adhésif (26) est optiquement transparente.

8. Procédé selon la revendication 5, dans lequel le film (20) est optiquement transparent.

9. Procédé selon la revendication 5, dans lequel la fixation du film de polymère (20) sur le substrat irrégulier (10) comprend l'établissement d'un contact seulement partiel entre la couche d'adhésif (26) et le substrat irrégulier (10).

10. Procédé selon la revendication 5, dans lequel l'impression d'une image (22) avec une encre à base de solvant comprend une impression au jet d'encre avec une encre à base de solvant.

11. Procédé selon la revendication 5, dans lequel le substrat irrégulier comprend une surface plane (12) et des éléments de surface non plans (14, 16).

12. Assemblage, comprenant :
un substrat irrégulier (10) comportant une surface non plane ;
une couche d'adhésif (26) en contact avec le substrat irrégulier (10) ;
un film de polymère (20) en contact avec la couche d'adhésif (26), le film de polymère (20) ayant une température de transition vitreuse d'au moins 40 °C ; et
une image (22) imprimée au jet d'encre avec un système piézoélectrique sur le film de polymère (20),
l'adhésif étant un adhésif sensible à la pression qui est collant aux températures d'assemblage.

13. Assemblage selon la revendication 12, dans lequel le film de polymère (20) a une température de transition vitreuse d'au moins 80 °C.
